

Oct. 2, 1928.

1,686,037

J. SCHNEPF

RESISTOR SUPPORT

Filed June 24, 1927

Fig.1.



Fig.2.



WITNESSES:

*Alspiegelheim.*  
*W. Salzman*

INVENTOR

*Johann Schnepf.*  
*Wesley Barr*  
ATTORNEY

## UNITED STATES PATENT OFFICE.

JOHANN SCHNEPE, OF NUEREMBERG, GERMANY, ASSIGNOR TO WESTINGHOUSE ELECTRIC &amp; MANUFACTURING COMPANY, A CORPORATION OF PENNSYLVANIA.

## RESISTOR SUPPORT.

Application filed June 24, 1927, Serial No. 201,289, and in Germany July 17, 1926.

My invention relates to electric furnaces and more particularly to means for supporting an electric resistance heating element therein.

5 In electric resistor furnaces, it is customary to support the resistor upon the walls by means of supports projecting from the faces thereof. In view of the relatively high temperatures attained in such furnaces, it is 10 necessary that the supports be made of a refractory heat-resistant material which is usually ceramic.

Ceramic refractory supports, however, are usually of an acid characteristic because of 15 the presence of silicic acid, and a chemical reaction between the support and metallic resistor results.

It is an object of the present invention, therefore, to provide in an electrical resistor furnace, means for preventing chemical reaction between the resistor and the resistor supporting means.

In one form of device embodying my invention, I provide an electrical resistance furnace comprising a metallic resistor supported by the walls of the heated chamber on refractory supports projecting therefrom, and a coating of material upon said supports for preventing chemical reaction between 30 said supports and said resistor.

In the drawings, Fig. 1 is a lateral section through a resistance furnace embodying my invention,

Fig. 2 is a view in longitudinal section 35 through a refractory resistor supporting block.

Referring more particularly to Fig. 1, the furnace embodying my invention comprises a plurality of built-up refractory walls 2 defining a furnace heating chamber 4.

Mounted in the side walls of said furnace chamber are a plurality of grooved supporting blocks 6, spaced to receive the upper ends of the convolutions of a preformed metallic 45 resistance heating element 8, in supporting relation. The resistance element is formed of metallic refractory material, and preferably of a nickel-chromium-iron alloy.

A plurality of refractory blocks 10 are 50 mounted in the furnace chamber side walls and are adapted to be received between the lower ends of the convolutions of resistor 8 to space the same along the furnace walls,

and prevent warping and consequent short circuiting thereof when heated.

As shown more particularly in Fig. 2 the resistor supporting block 6 is grooved in the upper face thereof to receive the resistor convolutions and is coated, upon the portion thereof to be exposed in the furnace chamber, with a refractory material 12 which has no chemical effect upon the metallic resistor.

Similarly, the spaced blocks 10 are coated to protect the lower portions of the resistor convolutions from chemical reaction with the acid refractory material.

The coating 12 may be of any suitable material which will not react chemically with the resistor and which has the necessary refractory qualities. In the present instance, I prefer to use zirconium oxide which may be formed thereon by depositing chemically or electrolytically upon the refractory supports, a coating of zirconium which is subsequently changed into the oxide by oxidation.

Another method of forming said coating upon the refractory support is to immerse the support in a solution of zirconium oxide powder which will penetrate into the pores 80 of the refractory.

With either of the above-described methods of coating the resistor support with the oxide, a close grained coating results which is sufficiently adherent to withstand the rough usage incident to furnace operation.

By my invention I have provided a means for preventing a chemical reaction between normally acid refractory resistor supports and the metallic resistors supported thereby.

While for purposes of description I have considered only a refractory support having an acid characteristic, it is clearly within the scope of the present invention to provide such a coating upon a refractory support having a basic characteristic if such characteristic produces a deleterious effect upon the resistor. Also, while I have shown a preformed sinuous resistor element and a specific shape of support obviously the shape or form of the resistor and of the refractory support is immaterial so far as the scope of the present invention is concerned.

Modifications may be made in my invention without departing from the spirit and scope thereof, and I desire therefore that

only such limitations be placed thereon as are imposed by the prior art and set forth in the appended claims.

I claim as my invention:

- 5 1. In an electric furnace, a resistance heating element, refractory means of normally acid characteristic directly supporting said resistance element within said furnace, and means for shielding said resistance element 10 from the deleterious effects occasioned by said acid refractory supports.
- 15 2. In an electric furnace, a resistance heating element, refractory means of normally acid characteristic for supporting said resistance element within said furnace, and a refractory coating of chemically neutral characteristic upon said supporting means for preventing chemical reaction between said resistance element and support.
- 20 3. In an electric furnace, a metallic resistance heating element, refractory supporting means therefor of a normally acid character-

istic, and a zirconium oxide coating formed upon said supporting means between said means and said resistance element for preventing chemical reaction therebetween.

4. In an electric furnace, an electric resistance heating element, refractory means directly supporting said element within said furnace, said means composed of a material which chemically reacts with said resistance element, and means between said support and said resistance element for preventing said chemical reactions.

5. In an electrically heated device, the combination with a metal resistor and a refractory support therefor, of a coating of zirconium oxide on said refractory support to prevent chemical reaction between said support and said resistor.

In testimony whereof, I have hereunto subscribed my name at Nuremberg this 13th day of May, 1927.

JOHANN SCHNEPF.